

## UNITED STATES PATENT OFFICE

2,126,000

## DRESSING TEXTILE THREADS

Henry Hans Freund, Cliffside Park, N. J., assignor to E. I. du Pont de Nemours & Company, Wilmington, Del., a corporation of Delaware

No Drawing. Application January 9, 1937, Serial No. 119,874

7 Claims. (Cl. 28—1)

This invention relates to the dressing of textile threads, particularly artificial threads such as threads formed from regenerated cellulose, cellulose derivatives and the like prior to weaving, knitting, or other fabrication thereof.

Artificial threads, particularly threads prepared from viscose, are inherently wiry, harsh, and non-pliable. Consequently, prior to fabrication into, for example, knitted fabrics, they must be softened and lubricated. Hitherto, animal or vegetable oils in combination with paraffin oils have been used as dressing, softening, or lubricating compositions for textile threads. While paraffin oils alone are unsatisfactory for dressing textile yarns inasmuch as they soften the yarn to only a very slight degree and are removed from the yarn only with a great deal of difficulty, it is desirable to add a certain amount of such an oil to vegetable or animal oil compositions in order to get a desirable viscosity, easy penetration of oil into the textile yarn and a reduction in the quantity of the expensive animal or vegetable oil used. Furthermore, animal and vegetable oils are susceptible to oxidation, which deleteriously affects the yarn treated with these oils. It has, therefore, been found desirable to use only as much of the oxidizable oil as will give a satisfactory softening of the yarn.

It is therefore an object of this invention to provide an improved dressing composition for textile threads. Another object is to provide textile fibers or threads, particularly artificial threads, such as those formed from regenerated cellulose, cellulose derivatives and the like, dressed with an improved dressing composition. A further object is to provide a dressing composition that produces a very satisfactory softening and lubrication action and at the same time can be easily and substantially completely removed from the thread. Other objects will appear hereinafter.

The objects of this invention are in general accomplished by dressing textile fibers or threads, particularly artificial threads such as regenerated cellulose, cellulose derivatives and the like, with a composition comprising naphthenes and one or more animal or vegetable oils.

Naphthenes in general are saturated cyclic hydrocarbons and are contained in many of the mineral oils from all parts of the world. They are predominant in the Russian oils such as from Baku, German oils such as from Wietze, Roumanian oils, and oils from certain South American countries such as Argentina. They occur

to some extent in almost every crude natural oil.

Naphthene oils are now available in commercial form such that the product contains no more than 2 or 3% unsaturated materials and with a suitable viscosity at boiling point range as to make them eminently suited as components in thread dressing composition. It is desirable that the crude oil containing the naphthene be carefully fractionated within reasonably narrow boiling limits so as to produce a product free from very light and very heavy fractions. The selected fractions of naphthenes are desired for the dressing of textile yarns because they can be more readily removed with a smaller amount of emulsifying agent in the boil-off than if the fractionating were not so carefully done.

The naphthene oil composition which has given the most satisfactory results has the following characteristics:

Boiling point range: 550° F. to 715° F.

Saybolt viscosity at 100° F.: 65 seconds

Unsaturated matter: Less than 3%

Pour test: —60° F.

Color: Substantially none.

Other naphthenes, however, may also be used such as those boiling in the range 500° F. to 800° F. or having a viscosity between 50 and 75 seconds at 100° F. or even outside these limits. The naphthenes which can be satisfactorily used depend upon the textile thread, the animal or vegetable oil used and many other factors.

The naphthenes herein described may be used in combination with any of the animal or vegetable oils commonly used as softening or lubricating agents, such as, olive oil, cotton seed oil, castor oil, palm oil, cocoanut oil, neat's-foot oil, lard oil, and the like. Instead of animal or vegetable oils, there may be used sulfonated animal or vegetable oils or mineral oil sulfonates. The proportion of naphthenes in the compositions should in general be from 50-80%, or more.

There may also be included in the compositions anti-oxidants for the animal or vegetable oil such as beta-naphthol, diphenylamine and the like. The amount of animal or vegetable oils used may also be reduced to some extent by the addition of a phosphatide such as lecithin in an amount from 0.1 to 3.0% or more of the total composition, in order to improve the softening power of the animal or vegetable oil and render the treated thread more supple.

To more clearly explain this invention there are hereinafter set forth specific illustrative com-

20

25

30

35

40

45

50

55

positions which are suitable for dressing artificial threads formed of regenerated cellulose or cellulose acetate:

*Example I*

|               | Percent |
|---------------|---------|
| Olive oil     | 35      |
| Naphthene oil | 65      |

*Example II*

|               | Percent |
|---------------|---------|
| Olive oil     | 15      |
| Palm oil      | 10      |
| Lecithin      | 0.5     |
| Beta-naphthol | 0.1     |
| Naphthene oil | 74.4    |

15 Since naphthenes in general have greater penetrating power than paraffin oils, yarn treated with these compositions is somewhat softer than that obtainable by using similar compositions wherein 20 paraffin oil is used in place of the naphthene oil. Furthermore, yarns so dressed can be readily knit at high speeds with a higher number of stitch count than is possible with the prior art compositions containing paraffin oil.

25 Though the invention has been described in connection with artificial threads formed of regenerated cellulose, cellulose acetate, etc., the invention is not restricted thereto. It is equally applicable to all textile threads.

30 The dressing composition may be applied to the yarn in any suitable manner. In the preferred mode of use, the composition is intermittently or continuously applied to the yarn while it is being wound in suitable packages, for example, cones, by appropriate mechanical devices such as those used on winding machines for oiling thread.

35 Since it is obvious that various changes may be made in the specific details hereinabove set forth,

this invention is not restricted thereto except as set forth in the appended claims.

I claim:

1. Textile threads dressed with a composition comprising at least 50% unsubstituted naphthenes and at least one material taken from the class consisting of animal oils, vegetable oils, sulfonated animal oils, sulfonated vegetable oils, and sulfonated mineral oils. 5

2. Textile threads dressed with a composition comprising an animal oil and at least 50% unsubstituted naphthenes. 10

3. Textile threads dressed with a composition comprising a vegetable oil and at least 50% unsubstituted naphthenes. 15

4. Artificial textile threads dressed with a composition comprising at least 50% unsubstituted naphthenes and at least one material taken from the class consisting of animal oils, vegetable oils, sulfonated animal oils, sulfonated vegetable oils, 20 and sulfonated mineral oils.

5. Regenerated cellulose threads dressed with a composition comprising at least 50% unsubstituted naphthenes and at least one material taken from the class consisting of animal oils, vegetable 25 oils, sulfonated animal oils, sulfonated vegetable oils, and sulfonated mineral oils.

6. A composition for dressing textile threads comprising at least 50% unsubstituted naphthenes and at least one material taken from the 30 class consisting of animal oils, vegetable oils, sulfonated animal oils, sulfonated vegetable oils, and sulfonated mineral oils.

7. Textile threads dressed with a composition comprising at least 50% unsubstituted naphthenes. 35

HENRY HANS FREUND.